

# UNITED STATES PATENT OFFICE.

OLOF JONATHAN MELLGREN, OF GOTTFENBORG, SWEDEN.

## METHOD FOR THE MANUFACTURE OF IGNITING COMPOSITIONS FOR MATCHES.

1,379,355.

Specification of Letters Patent. Patented May 24, 1921.

No Drawing.

Application filed November 11, 1919. Serial No. 337,140.

To all whom it may concern:

Be it known that I, OLOF JONATHAN MELLGREN, a subject of the King of Sweden, residing at Gottenborg, in the county of 5 Gottenborg and Bohus and Kingdom of Sweden, have invented a Method for the Manufacture of Igniting Compositions for Matches and Matches Manufactured by This Method, of which the following is a specification.

This invention refers to the manufacture of matches and has for its object to provide means for making such matches cheaper without interfering with their good character.

The present invention consists in a method to partly substitute one or more of the components of the igniting head of the match by a cheaper product, thereby maintaining or increasing the advantageous qualities of the head.

The igniting head of matches generally is composed partly by elements with high igniting properties (for instance potassium 25 chlorate and similar substances) for starting the ignition, when the match is struck against the friction surface, partly by elements which fill up the composition and modify the kindling of the match, and 30 partly by elements for binding the different components in the head. Besides there are present some mediums for saturating and coloring the head.

The filling substances must dilute the 35 igniting composition, to obtain suitable inflammability. In other words the head of the match has to be inflammable without tendency to throw sparks. The binding substances must join the different components in the head together without decreasing the igniting ability. In order to obtain suitable ingredients for the head, it is necessary to use composing elements of the very best quality, which generally means 40 a high price of manufacture. It is therefore obvious, that, if one or more of the elements heretofore used could be substituted partly or wholly by elements of a cheaper product without decreasing the 45 high quality of the head, it would mean a considerable saving in costs.

It has heretofore, for instance in the Smith Patent No. 3773, been proposed to employ pulverized vegetable matters of all kinds, 55 such as wood, bark, etc., as a component in the igniting composition of friction matches,

and preferably vegetable matters, containing tannin, for instance oak bark, nut-galls, the tannin serving to form with glue or gelatinous matters a substance, which will 60 have an advantageous effect on the igniting composition.

It has however, been proved, that all vegetable matters will not suit the purpose, because it is of very great importance, that 65 the matter used have certain properties not found in any of the vegetable matters, proposed in the Smith patent.

The object of the present invention is to substitute part of the glue, as a component 70 in the igniting composition of matches, with an ingredient which, by a special grinding process can be ground into an extraordinarily fine state. The substance referred to is the bark of *Pinus Silvestris*, 75 which containing practically no tannin nevertheless serves as a good binder on account of its percentage of resinous substance, so that the expansive gluey substances can be dispensed with in an essential 80 degree. Moreover this material (bark from *Pinus Silvestris*) when in finely divided and purified state has a property of still greater importance for the igniting composition. The cells of the bark of *Pinus Silvestris* 85 consists of resinous walls inclosing air. The percentage of air required in igniting composition of high quality is obtained by the use of these cells.

The bark, which in dry condition has a 90 specific gravity of 0.325, is ground, so that the powder finally obtained has a net weight of 24½ lbs. per cub. foot when loosely filled in a vessel. The air inclosed in the cells of the bark giving the effect, that the combustion takes place in a very quiet and secure but at the same time powerful way.

By adding more or less of the powder of pinebark the inflammability of the igniting composition may be regulated in a very 100 convenient and safe way.

What is claimed as new is:—

1. In the manufacture of igniting composition for matches, the substituting of part of binding materials hitherto used as 105 part of the igniting composition for matches by the powder of tree bark which in every respect has the properties for substituting gluey substances, and at the same time supplying the igniting composition with air, 110 for the purpose set forth.

2. In the manufacture of igniting com-

position for matches, the substituting of part of binding materials hitherto used as part of the igniting composition for matches by the powder of bark from *Pinus Silvestris* as and for the purpose set forth.

3. In an igniting composition for matches, binding material including a resinous substance in powdered form and having air filled cells.

10. 4. In the manufacture of igniting composition for matches, the substitution of part of the binding materials heretofore

used, by resinous bark divided into fine state without destroying the air filled cells of the bark.

5. In the manufacture of igniting compositions for matches, the substituting of part of the binding materials heretofore known by the powder of a bark having substantially the same properties as the bark of *Pinus Silvestris*.<sup>15</sup>

In testimony whereof I have affixed my signature.

OLOF JONATHAN MELLGREN.